

## UNITED STATES PATENT OFFICE

CHARLES S. SHELTON, OF SEATTLE, WASHINGTON

## WATERPROOFING COMPOSITION

No Drawing.

Application filed April 18, 1925. Serial No. 24,262.

This invention relates to paper waterproofing compositions.

The primary object of the invention is the provision of a composition of this character which is inexpensive to manufacture and readily applied.

A further object of the invention is the provision of a waterproofing composition which will serve as a preservative to render paper practically immune to the destructive effects of atmospheric and temperature changes.

A still further object is the provision of a waterproofing composition for treating paper without rendering the same hard and brittle.

The invention consists of a mixture of a metallic oxide, benzol, petroleum-ether, and a pliant cementatory material, such as dammar or other resinous gum, having similar characteristics, silicate of sodium or silicate of potassium.

Although I do not wish to limit myself to any specific proportions in preparing the composition I prefer to use the ingredients in about the following proportions, by bulk, viz: metallic oxide, sixteen parts; gum, four parts; benzol, seventy-four parts; and petroleum-ether, eight parts. Instead of the resinous-gum good results are obtainable by substituting therefor a like quantity of silicate of sodium or potassium (soluble glass).

The ingredients of my waterproofing composition are mixed together producing a liquid mass ready for use.

In applying the composition to paper, the latter is advantageously immersed in a quantity of the composition.

The functions of the various components may be explained as follows: The benzol serves as a diluting agent with respect to the metallic oxide, that is to say, to produce a fluid mixture of the oxide and benzol; said benzol also acts upon the paper material or stock to cause the same to have an affinity for the composition as a whole thereby permitting its entering the minute pores of the paper to thoroughly permeate the latter; the oxide serves as a metallic filler for the paper; the gum (or silicate) serves as a cementatory

substance; and the petroleum-ether serves as a drier.

The metallic oxide employed in my composition would be of a kind suitable to a particular grade of paper stock for obtaining various results—such oxide being, for instance, either oxide of lead, or oxide of zinc, or a mixture of the lead or zinc oxide with oxide of lead in the proportion of about four to one.

An aromatic substance—as anise oil, for example—may be employed for use with certain grades of paper.

What I claim, is—

1. A composition for waterproofing paper comprising a preparation comprising approximately twelve parts of oxide of zinc, three parts of oxide of lead, and five parts of dammar gum, with about eighty-two parts of a liquid consisting of benzol and petroleum-ether.

2. In treating paper to render same non-absorbent of moisture throughout its entire thickness, a composition, said composition comprising the solids zinc oxide and dammar gum, and the fluid components benzol and petroleum ether, said solids and fluids being in substantially the proportion of one to four.

Signed at Seattle, Washington, this 9th day of April, 1925.

CHARLES S. SHELTON.

55

60

65

70

75

80

85

90

95

100